

A. L. CLAPP.  
PUFFED PAPER IMITATING FELT AND PROCESS OF MAKING THE SAME.  
APPLICATION FILED JULY 25, 1911.

1,038,086.

Patented Sept. 10, 1912.

Fig. 1.



Fig. 2.



Witnesses:

Peter Jr. Pezzetti  
Forest R. Bonellone

Inventor:  
Albert L. Clapp  
by myself, Donald L. May  
Attest

# UNITED STATES PATENT OFFICE.

ALBERT L. CLAPP, OF BRAINTREE, MASSACHUSETTS, ASSIGNOR, BY MESNE ASSIGNMENTS, TO A. LEON CUTLER, OF BOSTON, MASSACHUSETTS.

## PUFFED PAPER IMITATING FELT AND PROCESS OF MAKING THE SAME.

1,038,086.

Specification of Letters Patent. Patented Sept. 10, 1912.

Application filed July 25, 1911. Serial No. 640,505.

To all whom it may concern:

Be it known that I, ALBERT L. CLAPP, a citizen of the United States, and a resident of Braintree, in the county of Norfolk and State of Massachusetts, have invented certain new and useful Improvements in Puffed Paper Imitating Felt and the Process of Making the Same, of which the following is a specification.

10 I have made a peculiar and what I believe to be an original product from sheets of wood pulp, kraft, sulfite pulp and other forms of disintegrated or beaten-out cellulose fibers. This product I have called paper 15 felt or puffed pulp.

In carrying out this process wood pulp, preferably that of a fibrous nature as sulfite pulp, kraft paper, or kraft pulp in sheet form is immersed in a strong solution of 20 caustic soda ( $NaOH$ ), about a twenty or twenty-five per cent. solution being well adapted for the purpose. Care must be taken not to let the sheet remain so long in the solution as to disassociate the fibers 25 and cause them to fall apart under the strong disintegrating action of the solution, the object being to retain the pulp or fibers in sheet form throughout the process. When the solution is of about the strength above 30 specified the period of immersion may be about two minutes.

The sheets may be immersed by any suitable means, as by placing them on a wire gauze bed adapted to be lowered into the 35 solution and raised therefrom, or to pass horizontally through the solution. As soon as the sheet is saturated with the solution and before it can be disintegrated it is removed and exposed to air to dry. For this 40 purpose the sheet may be laid out on a flat bed of wire gauze or other foraminous material permitting free access of air to the under side of the sheet, its upper side being at the same time exposed to the air. The 45 sheet may be hung in a chamber and dried by air forced into the chamber and preferably heated. There are, however, many practical ways of drying, it being necessary only to surround each sheet with a constant 50 and fresh supply of air. The importance of air drying will be readily seen from what follows in this description.

As the sheet of pulp which is still saturated with the strong soda solution begins 55 to dry, the caustic soda ( $NaOH$ ) is convert-

ed into sodium carbonate ( $Na_2CO_3$ ) due to the absorption of carbon dioxide from the air, and as this absorption increases, the fibers swell or puff to many times their natural size. When the chemical action is completed and the sheet is practically dry, the product has very much the appearance and general properties of felt, the fibers being sufficiently matted to hold together in the form of a sheet. There still remains throughout the sheet a considerable quantity of alkali in the form of crystals of sodium carbonate which discolors or imparts a whitish tinge to the sheet and requires removal to render the product commercially useful as a substitute for felt. This is accomplished by rapidly passing the dried sheet through a neutralizing bath of sulfuric or other suitable acid, a sulfuric acid solution ranging from five to ten per cent. being suitable, and the period of immersion in the neutralizing bath being relatively brief. It is now necessary to dry the sheet again, but at this stage of the process it is not necessary to have so plentiful an air supply as before because there is no further chemical action. When the sheet is finally dried, it still retains the physical appearance of a sheet of felt and may be dyed to any color.

The puffing process is not confined to the use of a solution of caustic soda although this has been found in general practice to be the most suitable chemical. Other chemicals which are soluble in water and will change chemically when exposed to the action of air may be used, such as sodium sulfite, caustic potash and certain iron salts. It is this chemical action resulting when caustic soda is employed, in the absorption of carbon dioxide from the air which causes the fibers to swell or puff. The capillary cells of the fibers saturated with a strong chemical solution having an affinity for elements of the air, inevitably swell as the absorption of the elements increases.

It will be seen from the foregoing that the puffing or swelling is dependent upon a sufficient supply of air to cause the fibers to puff quickly and evenly. The thickness of the puffed sheet is regulated by the strength of the puffing solution and by the original thickness of the sheet.

Figure 1 of the accompanying drawing represents in perspective a sheet which has

not been treated; Fig. 2 represents in perspective the same sheet puffed in accordance with my invention, the sheet being increased to several times its original thickness and its area somewhat decreased.

The texture of the surfaces of the sheet is changed by the process so that the sheet closely resembles felt.

I claim:—

10 1. As an article of manufacture a sheet composed of associated wood fibers puffed or increased in diameter, the sheet having a surface texture resembling felt.

15 2. The process of puffing and felting wood fibers associated in sheet form, the same consisting in saturating the sheet with a chemical solution having an affinity for elements of the air, and then subjecting the saturated sheet to contact with air until the 20 fibers are puffed or increased in diameter and the sheet acquires a surface texture resembling felt.

25 3. The process of puffing and felting wood fibers associated in sheet form, the same consisting in saturating the sheet with an alkaline solution having an affinity for elements of the air, then subjecting the sheet to con-

tact with air until the fibers are puffed or increased in diameter and the sheet acquires a surface texture resembling felt, and finally 30 neutralizing the crystallized alkali.

4. The process of puffing and felting wood fibers associated in sheet form, the same consisting in saturating the sheet with a solution of caustic soda, and then subjecting the 35 saturated sheet to contact with air until the fibers are puffed or increased in diameter and the sheet acquires a surface texture resembling felt.

5. The process of puffing and felting wood 40 fibers associated in sheet form, the same consisting in saturating the sheet with a solution of caustic soda, then subjecting the saturated sheet to contact with air until the fibers are puffed or increased in diameter 45 and the sheet acquires a surface texture resembling felt, and finally subjecting the sheet to a neutralizing bath.

In testimony whereof I have affixed my signature, in presence of two witnesses.

ALBERT L. CLAPP.

Witnesses:

C. F. BROWN,  
OTIS M. CARTER.